

Feb. 27, 1940.

R. K. HOPKINS

2,191,477

## METHOD FOR MANUFACTURING CAST METAL BODIES

Filed Aug. 16, 1938



FIG. 1

FIG. 4

INVENTOR  
ROBERT K. HOPKINS  
BY *Virgil F. Davis*  
ATTORNEY

## UNITED STATES PATENT OFFICE

2,191,477

## METHOD FOR MANUFACTURING CAST METAL BODIES

Robert K. Hopkins, New York, N. Y., assignor to M. W. Kellogg Co., New York, N. Y., a corporation of Delaware

Application August 16, 1938, Serial No. 225,123

3 Claims. (Cl. 22—200)

This invention relates to the manufacture of metal bodies and in particular to the manufacture of cast metal bodies such as ingots, and the like.

5 Cast metal bodies of ferrous metals and alloys, and certain non-ferrous metals and alloys are seldom produced without imperfections in the metal at and adjacent the surface. These imperfections, cold shuts, folds, cracks, gas pockets etc., materially affect the quality of the metal, and, since they must be removed when it is desired to produce worked metal, they likewise seriously affect the cost of the final metal. The imperfections mentioned are always a source of 10 trouble and expense but particularly so when the ingot, or other cast body is of metal, such as chrome-steels, chrome-nickel steel, monel metal, nickel, etc., that are sluggish and do not flow freely in the molten condition. When the 15 metals, just mentioned, are cast the imperfections mentioned are generally more numerous than with the less sluggish and freer flowing metals and alloys. Also, due to the crystallization characteristics of the more sluggish metals coupled with the fact that these metals do not 20 usually readily weld during working operations, it is necessary to completely remove all of the defective metal as well as adjacent sound metal prior to working. This necessitates the removal 25 of a material proportion of the total ingot metal and generally is a major factor in the ultimate cost of the worked metal.

The imperfections at and adjacent the surface of the ingots such as cold shuts, folds, cracks, gas pockets, etc., are caused in the main by the chilling effect of the mold on the molten cast metal adjacent to the mold wall and are inherent in the present accepted mode of producing metal ingots and similar cast metal bodies.

40 I have found a simple and comparatively cheap way of eliminating, or at least materially lessening, the bad surface conditions inherent in accepted present day practice.

It is an object of this invention to provide a 45 method for producing cast metal bodies of superior surface characteristics in which the chilling effect of the mold on the molten cast metal is compensated for, so that its effects are substantially eliminated, or at least reduced to such 50 an extent that they do not materially affect the character of the surface metal of the cast body.

It is also an object of this invention to provide a 55 method for producing cast metal bodies of superior surface characteristics in which heat is added to the molten cast metal, adjacent the mold sides, during the casting operation to compensate for the chilling effect of the mold.

The further objects and advantages of this 60 invention will be better understood from a consideration of the following description of a pres-

ent preferred mode of carrying my invention out in practice, taken with the accompanying drawing, in which,

Fig. 1 is a diagrammatic front view, partly in section of an arrangement of apparatus for carrying out the novel method,

Fig. 2 is a temperature curve illustrating the temperature conditions as they exist across the mold at the molten metal surface in the present practice, and

10 Figs. 3 and 4 are curves similar to that of Fig. 2 illustrating the temperature conditions obtained with the novel method.

When molten metal is cast into a mold, it is cast at such a temperature as to give the maximum yield of sound metal. The casting temperature is dependent upon the analysis of the molten metal, the character of the mold employed, the volume of metal to be cast, etc. In the practice of the prior art, while the bulk of the metal cast may remain at the casting temperature, or substantially so, for the required time interval, the metal at and adjacent the mold sides does not and by reason of its reduced temperature produces surface imperfections.

When molten metal is cast into a mold in accordance with the practice of the prior art, the metal adjacent the mold sides cools at a very rapid rate by reason of the heat absorbed by the mold sides, and quickly drops to temperatures much lower than the metal further removed from the mold sides. This is true of the metal at and adjacent the surface of the cast metal.

The curve of Fig. 2 illustrates the temperature gradient that normally exists, in the prior art practice at the surface of the cast metal as it is being poured. The metal between points A and B of the curve is all at substantially the same temperature. This temperature though somewhat lower than the casting temperature approaches the pouring temperature so that the metal between points A and B is in the condition to produce a maximum of sound metal. The bulk of the metal represented by portions A—C and B—D of the curve is, however, at temperatures much below the casting temperature. The metal adjacent points C and D may actually be at or closely approach the solidification temperature of the metal. Thus, the metal between points A and C and B and D is not in the condition required for the production of sound metal

45 as it is cooled to such a degree that its fluidity is impaired. The required fluidity of the surface metal is responsible for the formation of cold shuts, folds, cracks, gas pockets, impurity 50 segregations, etc., in and adjacent the surface of the cast body.

55 In some cases the fluidity of the surface metal is so reduced that the later cast metal can only pass to the mold sides by passing through or over the cooled surface metal in 60

waves or surges thus, resulting in cold shuts, cracks, etc., between the wave fronts.

These imperfections are formed, for the reasons stated, even with metals such as carbon steel that are comparatively free flowing in the molten condition. When metals, ferrous alloys such as chrome steels, chrome-nickel steels (with or without various percentages of molybdenum and columbium), pure metals such as nickel, non-ferrous alloys such as monel metal, that do not flow readily at temperatures that tend to approach the solidification temperatures, and for that reason are generally designated as sluggish, are cast, the imperfections mentioned always occur to a troublesome extent.

The cooling effect of the mold sides may be compensated for, in accordance with my invention, by the addition of heat during the pouring of the metal so that the metal at and adjacent the mold sides will retain the necessary characteristics to produce imperfection free, or substantially imperfection free surfaces.

I supply the heat, preferably by means of discharge of electric current from the end of one or more electrodes, to the surface of the molten metal in such quantity and at such location that the temperature of the bulk of the metal at and adjacent the mold sides is brought to temperatures approaching or even higher than the temperatures of the remainder of the surface metal.

In the casting operation illustrated by the curve of Fig. 3 heat has been added to portions A'—C' and B'—D' of the surface metal and the quantity of heat added so controlled that the portion of substantially uniform temperature extends from point E to point F, the temperature at points C' and D' being raised by the heat addition until they approach the temperatures of the main part of the curve. Thus, the metal at and adjacent the walls of the mold is at a sufficiently high temperature that it has the required flow and other characteristics to produce a substantially imperfection free surface. This heat will usually be added at a point or region between the sides of the mold and the point at which the temperature begins to drop in the old practice. The exact location of the point or region mentioned will depend on many factors such as conduction of the molten metal, conduction and design of the mold etc., and is best arrived at in each particular case from experiment. The quantity of heat added will also vary but in any case will be such to render the metal at and adjacent the mold sides of sufficient fluidity that it will conform to the shape of the mold without appreciable resistance and will allow gas and solid impurities to pass through it.

In the operation illustrated by the curve of Fig. 4 the heat is added between points C''—A'' and B''—D'' as before but the quantity of heat added and the point or region of application is such that the temperature of the surface metal at and adjacent the sides of the mold is raised above the temperatures of the rest of the surface metal. This manner of operation is particularly satisfactory when casting very sluggish metal.

In order to secure satisfactory results it is necessary that the heat be applied substantially uniformly over the whole outer band of the molten surface. This may be accomplished by use of a plurality of properly spaced electrodes or by the use of one or more electrodes that are moved, either by their movement or by the movement

of the mold, at a substantially uniform rate over the portion of the surface metal to be heated.

When the electrode or electrodes are located close to the mold walls and the usual cast iron molds are employed there is the possibility that the mold walls may be fused and united to the cast metal. To remove this possibility the mold, or the inside portions thereof, may be made of a metal or alloy of high heat conductivity such as copper, copper alloys, etc., and provided with a jacket through which water, oil, or other heat exchange medium may be circulated. In lieu of a jacket the mold may include passageways within it through which the heat exchange medium may be circulated. The jacket or the passageways may be so arranged that the whole of the mold may be cooled at one time or only selected horizontal bands may be cooled as desired. With the latter arrangement and especially when normal cooling of the cast metal is desired, that portion of the mold only can be cooled at which the heat is being applied also, the mold may be made of refractory material that will withstand the heat of the current discharge.

The electric discharge may take place from the end of a non-consumable electrode, or electrodes, or from the end of a consumable electrode, or electrodes, of substantially the same composition as the cast metal. The electric discharge may be in the form of an open arc but more satisfactory results are obtained when the surface of the molten metal, the electric discharge and the end of the electrode, or electrodes, are maintained beneath a thick blanket of protective flux. The thickness of the blanket may range from  $\frac{1}{2}$ " to 6" or more depending on the size of mold, intensity of discharge etc.

The flux may be initially solid or molten and additions may be made as required. The slag produced in the making of the molten metal may be employed as the flux or any suitable material that will protect the electric discharge and the molten metal from the atmosphere, will not add undesirable constituents or remove desirable constituents, and will not produce deleterious gas either as to quantity or kind may be employed. At present, silicates of calcium, magnesium, manganese and iron, either alone or in mixture, or their unreacted dried or calcined components are preferred fluxes. The flux may also contain aluminates, titanates, flux thinners such as fluor-spar etc.

The illustrative form of apparatus, suitable for carrying out the novel method of the invention, diagrammatically shown in Fig. 1, includes a mold 10 which may be arranged for either top pouring or bottom pouring of the molten metal. Mold 10 may be of any desired construction; thus, it may be of the big end up type or the big end down type and may be made of cast iron, as in the usual practice or of copper, and the like, and provided with a jacket or similar means through which water or other heat exchange medium may be circulated. Mold 10 may also be of refractory materials, in which case the water circulating means are omitted. Mold 10, as shown, includes a plurality of passageways 11 through which a heat exchange medium may be circulated. Passageways 11 may be connected into a continuous flow path for the heat exchange medium or they may be so arranged in connectable horizontal coils that the heat exchange medium can be circulated at will through one or more of them to cool desired horizontal sections of the mold.

Mold 10 may be supported on a fixed stand or it may be supported on rotatable means for rotation about a vertical axis. When top pouring is employed the molten metal passes from ladle 12 through a suitable conduit 13 to discharge into the mold beneath flux blanket 14. When bottom pouring is resorted to the molten metal is supplied from a ladle 15 to a suitable conduit 16 that opens in the bottom of the mold and discharges the molten metal beneath flux blanket 14.

Shortly after the casting operation is initiated electric current is discharged from the end of electrode 17 to the surface of the molten metal 18. The end of the electrode as well as the electric discharge is maintained beneath the blanket of flux 14. Electrode 17 is fed by feed wheels 19 through a contact nozzle 20 to the surface of the molten metal 18 at the required rate to maintain a discharge of predetermined characteristics. This result is obtained by reason of the control arrangements located in welding head 21. Head 21 may be of any of the types well known in the arc welding art. Current is supplied to contact device 20 through cable 22; cable 23 conducts the current to the mold 10.

Welding head 21 may be arranged to carry electrode 17 around the mold or it may be fixed in position. While only one electrode 17 has been shown, it is to be understood that as large a number may be used as is found necessary in order to obtain the desired heat input to the whole body of surface metal at and adjacent the mold sides. As stated, the electrode, or electrodes, may be moved around the mold or they may be maintained in fixed position and the mold rotated. Also, both molds and electrodes may be fixed. In such case a plurality of closely spaced electrodes are employed.

While the welding head 21 will raise the end of electrode 17 as required to maintain the desired discharge, it is advisable to provide means, either manual or automatic for raising head 21 with the rising level of molten metal 18 to prevent injury by the heat to contact device 20 and head 21. When mold 10 is not of constant cross section provision must also be made to move head 21 and electrode 17 laterally so that the discharge end of electrode 17 may be maintained at the predetermined distance from the sides of mold 10. As heretofore stated, the location of the discharge and its intensity depends on the characteristics of the metal cast, the size and design of the mold, etc. To obtain the desired results it will often be necessary to locate the discharge near the mold walls. In such cases the mold will be of refractory material or it may be made of copper or similar high heat conductivity metal and a cooling medium circulated through passageways 11. The whole of the mold may be cooled simultaneously or only the horizontal zone thereof adjacent the level of the molten metal 18.

The molten metal may be supplied entirely from ladles 12 and 15 or only some of it may be so supplied and the remainder supplied from one or more electrodes of the required composition. Also, ladles 12 and 15 may be dispensed with and all of the molten metal supplied from one or more electrodes. When electrodes are employed their discharge will also be maintained beneath flux blanket 14. The feed motors, control arrangements of these electrodes may be incorporated in head 21 or a separate head may be provided.

In the usual case the desired results are obtained, as explained above, by the addition of

the required heat to the surface metal at and adjacent the mold sides. In some cases, however, the desired results may be obtained by the addition of heat to substantially the whole of the surface metal, the heat being added in such quantity and in such manner to compensate for the chilling of the surface metal during the casting.

In these cases the heat may be added by the use of electrodes 17, as heretofore, but heat is also added to the center surface metal, i. e., the metal between points A and B of the curve of Fig. 2, so that the whole of the surface metal is raised above the temperatures of the prior practice, as represented by the curve of Fig. 2. Thus, in addition to electrodes 17, electrodes may be positioned at the center of the surface or somewhere between the center and electrodes 17.

In cases where the amount of heat required to compensate for the chilling of the surface metal is comparatively small electrodes 17 may be eliminated and all of the heat supplied by additional electrodes.

When the whole or a part of the cast metal is obtained, as pointed out above, by the fusion of consumable electrodes, the consumable electrodes may be so operated to supply a part or all of the compensating heat required.

As with electrodes 17, the additional electrodes may be non-consumable or consumable. In the latter event they are made of such composition to provide fused metal of the same composition as the cast metal. The discharge, or discharges, from the additional electrodes is also submerged beneath flux blanket 14.

I claim:

1. The method of casting metal bodies which comprises, placing a depth of protective flux in the bottom of a mold, casting molten metal into said mold beneath said flux to progressively fill said mold, discharging electric current from one or more electrodes against the rising molten metal surface adjacent the sides of said mold, said electric discharge being maintained beneath said blanket of flux and being of an intensity to maintain the surface metal at and adjacent the mold sides in substantially the same degree of mobility as the remainder of said surface metal.

2. The method of casting metal bodies made of metal of a melting point within the melting point range of ferrous alloys, which comprises, placing a depth of protective flux in the bottom of a metal mold, casting molten metal into said mold beneath said flux to progressively fill said mold, and discharging electric current from one or more electrodes against the rising molten metal surface adjacent the sides of the mold to maintain the molten surface metal adjacent the mold sides at temperatures approaching the pouring temperature.

3. The method of casting metal bodies made of metal of a melting point within the melting point range of ferrous alloys, which comprises, placing a depth of protective flux in the bottom of a metal mold, casting molten metal into said mold beneath said flux to progressively fill said mold, discharging electric current from one or more electrodes against the rising molten metal surface adjacent the sides of the mold to maintain the molten surface metal adjacent the mold sides at temperatures approaching the pouring temperature, and cooling the mold to prevent the molten metal fusing thereto.